# EUROPEAN PATENT SPECIFICATION

(11) **EP 3 821 046 B1**
(45) Date of publication and mention of the grant of the patent: **09.04.2025**
(21) Application number: 19746289.8
(22) Date of filing: 12.07.2019
(51) Int. Cl.: C22C 9/06, C22F 1/08, C22F 1/00, H01B 1/02

(54) **COPPER-NICKEL-SILICON ALLOYS WITH HIGH STRENGTH AND HIGH ELECTRICAL CONDUCTIVITY**
KUPFER-NICKEL-SILICIUM-LEGIERUNGEN MIT HOHER FESTIGKEIT UND HOHER ELEKTRISCHER LEITFÄHIGKEIT
ALLIAGES CUIVRE-NICKEL-SILICIUM PRÉSENTANT UNE RÉSISTANCE MÉCANIQUE ÉLEVÉE ET UNE CONDUCTIVITÉ ÉLECTRIQUE ÉLEVÉE

(30) Priority: 12.07.2018 US 201862696915 P
(43) Date of publication of application: 19.05.2021
(73) Proprietor: Materion Corporation, Mayfield Heights, OH 44124 (US)
(72) Inventor: TRYBUS, Carole L., Mayfield Heights, Ohio 44124 (US); KULI JR., John C., Mayfield Heights, Ohio 44124 (US); TAYLOR, Christopher J., Mayfield Heights, Ohio 44124 (US)
(74) Representative: Kador & Partner Part mbB
(86) International application number: PCT/US2019/041556
(87) International publication number: WO 2020/014582

(56) References cited:
- JP-A- 2003 257 417
- JP-A- 2008 223 069
- JP-A- 2014 074 202
- JP-A- H06 184 680
- US-A1- 2011 038 753

## Description

### CROSS-REFERENCE TO RELATED APPLICATIONS

### BACKGROUND

The present disclosure relates to copper alloys with a combination of high yield strength and high electrical conductivity. Processes for making and using such alloys are also disclosed, as well as articles produced therefrom.

Copper alloys with a combination of relatively high 0.2% offset yield strength and high electrical / thermal conductivity are difficult to achieve. Copper-beryllium alloys have such properties, but there are many applications in which the presence of beryllium is undesirable. Hence, there is a need for additional copper alloys having such desired characteristics amongst others.

JP 2014-074202 A discloses an alloy comprising Ni, Si, Zr, optionally < 1.5% Cr, Mn and/or Zn, balance Cu. Such an alloy may be used for a mold material or an aircraft member.

### BRIEF DESCRIPTION

Disclosed herein are copper-nickel-silicon alloys with a combination of high 0.2% offset yield strength and high electrical / thermal conductivity. The alloys contain at least nickel, silicon, chromium, manganese, zirconium, and copper. The alloys are defined according to claim 1. Desirably, the alloys do not contain beryllium and/or other certain metals. The alloys are cold worked and then solution annealed to produce fine grain sizes, then aged to form a variety of precipitates such as NiSi and CrZrSi precipitates. This creates a dislocation network with precipitates that come out on the grain boundaries, locking in the fine grain sizes. In particular embodiments, the alloys have a 0.2% offset yield strength of at least 551 MPa (80 ksi) and an electrical conductivity of at least 48%IACS. Such alloys are useful in applications such as heat management and as high strength and performance electrical connectors, among others.

Disclosed herein are copper alloys, comprising: from 1.2 wt% to 1.4 wt% nickel; from 0.3 wt% to 0.4 wt% silicon; from 0.3 wt% to 0.4 wt% chromium; from 0.08 wt% to 0.12 wt% manganese; from 0.02 wt% to 0.06 wt%zirconium;; and balance copper; wherein the alloy has a 0.2% offset yield strength of at least 551 MPa (80 ksi) and a conductivity of at least 48% IACS.

The copper alloys generally do not contain beryllium, titanium, iron, cobalt, magnesium, or boron.

The copper alloys may have an ultimate tensile strength of at least 607 MPa (88 ksi). The copper alloys may have an elastic modulus of at least 138 GPa (20 million psi). The copper alloys may have a % total elongation of at least 8%. The copper alloys may have a ductility of at least 5% to 15%. The copper alloys may have a formability ratio of 0.4/1 or lower. The copper alloys may contain silicides formed from silicon, chromium, nickel, and manganese.

In some embodiments, the copper alloys have a 0.2% offset yield strength of at least 551 MPa (80 ksi), a conductivity of at least 48% IACS, and a % total elongation to break (TE) of at least 8%.

In other embodiments, the copper alloys have a 0.2% offset yield strength of at least 551 MPa (80 ksi), a conductivity of at least 49% IACS, and an ultimate tensile strength of at least 620 MPa (90 ksi).

Also disclosed herein are processes for making a copper alloy that does not contain beryllium and has a 0.2% offset yield strength of at least 551 MPa (80 ksi) and a conductivity of at least 48% IACS. The processes comprise: cold working a copper-nickel-silicon-chromium-manganese-zirconium alloy to a percentage of cold working (% CW) of 80% to 95%; solution annealing the cold-worked copper-nickel-silicon-chromium-manganese-zirconium alloy; and aging the solution-annealed copper-nickel-silicon-chromium-manganese-zirconium alloy to obtain the copper alloy with a 0.2% offset yield strength of at least 551 MPa (80 ksi) and a conductivity of at least 48% IACS.

The solution annealing may be performed at a temperature of 900°C to 1000°C for a time period of 5 minutes to 20 minutes.

The aging may be performed at a temperature of 400°C to 460°C for a time period of 6 hours to 60 hours. In more specific embodiments, the aging is performed at a temperature of 400°C to 460°C for a time period of 6 hours to 18 hours. The copper alloys formed by these processes are also disclosed.

Also disclosed herein are articles formed from a copper-nickel-silicon-chromium-manganese-zirconium alloy, wherein the alloy has a 0.2% offset yield strength of at least 551 MPa (80 ksi) and a conductivity of at least 48% IACS.

Amongst other things, the article can be a heat sink; an electrical connector; an electronic connector; a wiring harness terminal; an electric vehicle charger contact; a high voltage/current/power terminal contact; a power connector contact; a midplane connector; a backplane connector; a card edge connector; a photovoltaic system connector; an appliance power contact; a computer power contact; a heat spreader; a bushing or bearing surface; or a component for an electronic device or an electrical device.

Also disclosed are processes of using a copper-nickel-silicon-chromium-manganese-zirconium alloy that has a 0.2% offset yield strength of at least 551 MPa (80 ksi) and a conductivity of at least 48% IACS, comprising: stamping an article from a strip of the copper-nickel-silicon-chromium-manganese-zirconium alloy.

These and other characteristics of the disclosure are more particularly disclosed below.

### BRIEF DESCRIPTION OF THE DRAWINGS

The following is a brief description of the drawings, which are presented for the purposes of illustrating the exemplary embodiments disclosed herein.
**FIG. 1** is an optical view of a copper-nickel-silicon-chromium-manganese-zirconium alloy.
**FIG. 2** is an image of a copper-nickel-silicon-chromium-manganese-zirconium alloy obtained by backscattered-electron scanning electron microscopy (BSE SEM).
**FIG. 3** is a graph representing the 0.2% offset yield strength in MPa (ksi) on the left y-axis, and conductivity as a percentage of the International Annealed Copper Standard (% IACS) on the right y-axis, of a copper-nickel-silicon-chromium-manganese-zirconium alloy having been aged at 427 °C (800°F). Samples were aged at time intervals, indicated on the x-axis, of 3, 6, 12, 18, and 24 hours, and measurements were taken after aging for each time interval. The left y-axis runs from 0 to 689 MPa (0 to 100 ksi) at intervals of 68.9 MPa (10 ksi). The right y-axis runs from 0 to 60 % IACS at intervals of 10.
**FIG. 4** is a graph representing the 0.2% offset yield strength in MPa (ksi) on the left y-axis, and conductivity in % IACS on the right y-axis, of a copper-nickel-silicon-chromium-manganese-zirconium alloy having been aged at 435 °C (815°F). Samples were aged at time intervals, indicated on the x-axis, of 3, 6, 12, and 18 hours, and measurements were taken after aging for each time interval. The left y-axis runs from 0 to 689 MPa (0 to 100 ksi) at intervals of 68.9 MPa (10 ksi). The right y-axis runs from 0 to 60 % IACS at intervals of 10.
**FIG. 5** is a graph representing the 0.2% offset yield strength in MPa (ksi) on the left y-axis, and conductivity in % IACS on the right y-axis, of a copper-nickel-silicon-chromium-manganese-zirconium alloy having been aged at 441 °C (825°F). Samples were aged at time intervals, indicated on the x-axis, of 3, 6, 12, and 18 hours, and measurements were taken after aging for each time interval. The left y-axis runs from 0 to 689 MPa (0 to 100 ksi) at intervals of 68.9 MPa (10 ksi). The right y-axis runs from 0 to 60 % IACS at intervals of 10.

### DETAILED DESCRIPTION

A more complete understanding of the components, processes and apparatuses disclosed herein can be obtained by reference to the accompanying drawings. These figures are merely schematic representations based on convenience and the ease of demonstrating the present disclosure, and are, therefore, not intended to indicate relative size and dimensions of the devices or components thereof.

All ranges disclosed herein are inclusive of the recited endpoint and independently combinable (for example, the range of "from 2 grams to 10 grams" is inclusive of the endpoints, 2 grams and 10 grams, and all the intermediate values).

The present disclosure may refer to temperatures for certain process steps. It is noted that these generally refer to the temperature at which the heat source (e.g. furnace) is set, and do not necessarily refer to the temperature which must be attained by the material being exposed to the heat.

The present disclosure relates to copper alloys as defined in claim 1; they contain nickel, silicon, chromium, manganese, and zirconium. Such alloys have a 0.2% offset yield strength of at least 551 MPa (80 ksi) and a conductivity of at least 48% IACS, a combination of strength and electrical conductivity that is not readily available. This permits use in heat management applications. Desirably, the alloys are formable, stampable, and free of beryllium.

Nickel is present in the copper alloys in an amount of from 1.2 wt% to 1.4 wt% nickel.

Silicon is present in the copper alloys in an amount of from 0.3 wt% to 0.4 wt%.

Chromium is present in the copper alloys in an amount of from 0.3 wt% to 0.4 wt%.

Manganese is present in the copper alloys in an amount of from 0.08 wt% to 0.12 wt%.

Zirconium is present in the copper alloys in an amount of from 0.02 wt% to 0.06 wt%.

The balance of the copper alloy is copper, excluding impurities..

The copper alloys may also have some impurities, but desirably do not. Impurities include beryllium, titanium, magnesium, and boron. Some of these elements are sometimes added during processing for specific purposes. For example, boron and iron can be used to further enhance the formation of equiaxed crystals and also diminish the dissimilarity of the diffusion rates of Ni and Sn in the matrix during solution heat treatment. Magnesium can serve as a deoxidizer. In the manufacturing processes of the present disclosure, these elements are ideally not used. For purposes of this disclosure, amounts of less than 0.01 wt% of these elements should be considered to be unavoidable impurities, i.e. their presence is not intended or desired.

The Cu-Ni-Si-Cr-Mn-Zr alloys of the present disclosure are processed to take advantage of multiple strengthening mechanisms. The alloys are cold worked and then solution annealed to keep grains small and fine. The alloys are then aged to bring out a variety of precipitates. Those precipitates can include Ni-Si precipitates, Cr-Zr-Si precipitates, and/or Cr-Ni-Mn-Si precipitates. The cold working creates a dislocation network that that causes the precipitates to come out on the grain boundaries, which locks in the fine grain size. The processes of the present disclosure generally comprise (1) cold working the Cu-Ni-Si-Cr-Mn-Zr alloy; (2) solution annealing the cold-worked alloy; and (3) aging the solution annealed alloy.

Cold working is a metal forming process typically performed near room temperature, in which an alloy is passed through rolls, dies, or is otherwise cold worked to reduce the section of the alloy and to make the section dimensions uniform. This increases the strength of the alloy. The degree of cold working performed is indicated in terms of % reduction in thickness, or % reduction in area, and is referred to in this disclosure as %CW. In the present processes, the alloy is provided as initially cast, and is then cold worked to a %CW of 85% to 95%.

Solution annealing involves heating a precipitation hardenable alloy to a high enough temperature to convert the microstructure into a single phase. A rapid quench to room temperature leaves the alloy in a supersaturated state that makes the alloy soft and ductile, helps regulate grain size, and prepares the alloy for aging. Subsequent heating of the supersaturated solid solution enables precipitation of the strengthening phase and hardens the alloy. In the present processes, after cold working, the cold-worked alloy is solution annealed at a temperature of 900°C to 1000°C, or from 900°C to 950°C, or from 925°C to 975°C, or from 950°C to 1000°C, or from 925°C to 950°C, or from 9750°C to 1000°C. The solution annealing may take place over a time period of 5 minutes to 20 minutes, or from 5 minutes to 15 minutes, or from 5 minutes to 10 minutes, or from 10 minutes to 20 minutes, or from 10 minutes to 15 minutes, or from 15 minutes to 20 minutes.

Aging is a heat treatment technique that produces ordering and fine particles (i.e. precipitates) of an impurity phase that impedes the movement of defects in a crystal lattice. This hardens the alloy. In the present processes, after solution annealing, the alloy is aged at a temperature of 400°C to 460°C ( 752°F to 860°F), or from 415°C to 460°C, or from 430°C to 460°C, or from 415°C to 445°C, or from 445°C to 460°C. The aging may take place over a time period of 6 hours to 60 hours, or 6 hours to 30 hours, or 6 hours to 24 hours, or 40 hours to 56 hours, or 6 hours to 12 hours, or 6 hours to 18 hours It is noted that the aging can be performed in multiple steps, with the temperature of each step being within these stated ranges and the total time of the multiple steps being within these stated ranges. Desirably, the aging is performed in a 100% hydrogen atmosphere.

The resulting copper-nickel-silicon-chromium-manganese-zirconium (Cu-Ni-Si-Cr-Mn-Zr) alloy has a 0.2% offset yield strength of at least 551 MPa (80 ksi) and an electrical conductivity of at least 48% IACS. In some embodiments, the alloy has a combination of a 0.2% offset yield strength of at least 565 MPa (82 ksi) and an electrical conductivity of at least 49% IACS. The 0.2% offset yield strength is measured according to ASTM E8. In particular embodiments, the alloy has a 0.2% offset yield strength of at least 551 MPa (80 ksi) to 655 MPa (95 ksi), or at least 565 MPa (82 ksi), or at least 579 MPa (84 ksi). In some more specific embodiments, the alloy has an electrical conductivity of at least 48% IACS, or at least 49% IACS, or at least 50% IACS. In other embodiments, the alloy has an electrical conductivity of at least 48% IACS to 55% IACS.

The Cu-Ni-Si-Cr-Mn-Zr alloys of the present disclosure also have an elastic modulus of at least 138 GPa (20 million psi). The elastic modulus is measured according to ASTM E111-17. The elastic modulus may go up to 152 GPa (22 Msi). The Cu-Ni-Si-Cr-Mn-Zr alloys of the present disclosure may also have an ultimate tensile strength (UTS) of at least 607 MPa (88 ksi), or at least 620 MPa (90 ksi), or at least 634 MPa (92 ksi). The ultimate tensile strength is measured according to ASTM E8. The Cu-Ni-Si-Cr-Mn-Zr alloys of the present disclosure may also have a thermal conductivity of at least 200 W/m·K.

The Cu-Ni-Si-Cr-Mn-Zr alloys of the present disclosure may also have a % total elongation to break (%TE) of at least 5%, or at least 6%, or at least 8%, or at least 10%. This value measures how much the alloy can be stretched before it breaks, and is a rough indicator of formability. The %TE is also measured according to ASTM E8. Alternatively, the Cu-Ni-Si-Cr-Mn-Zr alloys of the present disclosure may have a ductility of at least 5% when measured at room temperature (22°C). In more particular embodiments, the alloys have a ductility of at least 5% to 15%.

The Cu-Ni-Si-Cr-Mn-Zr alloys of the present disclosure may alternatively have a formability ratio of 0.4/1 or lower. Good formability is usually measured by the formability ratio or R/t ratio. This specifies the minimum inside radius of curvature (R) that is needed to form a 90° bend in a strip of thickness (t) without failure, i.e. the formability ratio is equal to R/t. Materials with good formability have a low formability ratio (i.e. low R/t), in other words a lower R/t is better. The formability ratio can be measured using the 90° V-block test, wherein a punch with a given radii of curvature is used to force a test strip into a 90° die, and then the outer radius of the bend is inspected for cracks. The formability ratio can also be reported as the ratio of the formability in the longitudinal (good way) direction to the formability in the transverse (bad way) direction, or as GW/BW.

Any combination of the 0.2% offset yield strength, electrical conductivity, elastic modulus, ultimate tensile strength, %TE, ductility, and formability ratio discussed above is contemplated for the Cu-Ni-Si-Cr-Mn-Zr alloys of the present disclosure.

In particular embodiments, the Cu-Ni-Si-Cr-Mn-Zr alloys of the present disclosure have a 0.2% offset yield strength of at least 551 MPa (80 ksi), a conductivity of at least 48% IACS, a %TE of at least 10%, and a tensile modulus of at least 138 GPa (20 Msi).

In particular embodiments, the Cu-Ni-Si-Cr-Mn-Zr alloys of the present disclosure have a 0.2% offset yield strength of at least 551 MPa (80 ksi), a conductivity of at least 49% IACS, and a UTS of at least 620 MPa (90 ksi).

In particular embodiments, the Cu-Ni-Si-Cr-Mn-Zr alloys of the present disclosure have a 0.2% offset yield strength of at least 579 MPa (84 ksi), a conductivity of at least 49% IACS, a %TE of at least 8%, and a tensile modulus of at least 138 GPa (20 Msi).

In particular embodiments, the Cu-Ni-Si-Cr-Mn-Zr alloys of the present disclosure have a 0.2% offset yield strength of at least 551 MPa (80 ksi), a conductivity of at least 50% IACS, a %TE of at least 10%, and a tensile modulus of at least 138 GPa (20 Msi).

The Cu-Ni-Si-Cr-Mn-Zr alloys of the present disclosure have a combination of good yield strength and high electrical conductivity. The alloys can be provided as strip, wire, rod, tube, and bar. The alloys are also highly solderable and easily plated with other materials. Articles can be formed, for example, by stamping a strip into the desired shape of the final article or an intermediate shape that can be bent into the shape of the final article. The articles can be overcoated, for example with tin or gold or other materials, to provide additional desired properties, either before or after being formed.

The alloys can be used to make, for example, electrical connectors; electronic connectors, terminal contacts, or power contacts, where high strength and high electrical conductivity are desired. Examples of specific articles may include a heat sink in a cellphone; wiring harness terminals; electric vehicle charger contacts; high voltage/current/power terminal contacts; power connector contacts; midplane connectors; backplane connectors; card edge connectors; photovoltaic system connectors; appliance power contacts; computer power contacts; heat spreaders; bushing or bearing surfaces; and generally any component for an electronic device or an electrical device.

The following examples are provided to illustrate the alloys, processes, articles, and properties of the present disclosure.

### EXAMPLES

### EXAMPLE 1

A Cu-Ni-Si-Cr-Mn-Zr alloy was cast and processed as described above to obtain a strip with a width of 38.1 cm (15 inches). Its properties were measured at six (6) locations across the width of the inner and outer wraps, and then averaged. The values were 0.2% offset yield strength of 581 MPa (84.3 ksi), %TE of 10.4%, tensile modulus 145 GPa (21 Msi), and conductivity of 50.3% IACS. The R/t ratio was 0.4/1.

**FIG. 1** is an optical image of the alloy after processing. Typical grains and some indications of work are visible. Some Ni-Cr silicides are visible.

**FIG. 2** is a BSE SEM image. The dark spots are Cr-Ni-Mn-Si silicides. These silicides have particle sizes on the order of 100 nanometers to 200 nm. Their presence is unique, and their small size is unusual. It is noted that these silicides are not visible in **FIG. 1****.**

### EXAMPLE 2

A Cu-1.23Ni-0.38Si-0.23Cr-0.08Mn-0.02Zr alloy was cast, cold worked to a %CW of 85% to 95%, solution annealed at a temperature of 900° to 1000°C, and then aged twice. The first aging was performed for 24 hours at either 800°F, 815°F, or 825°F (427°C, 435°C, 441°C). The second aging was performed for six hours at 800°F (427°C). The 0.2% offset yield strength (YS) and the electrical conductivity (%IACS) of the alloy were measured at various time points during the second aging, and are illustrated in three graphs.

**FIG. 3** shows the measured YS and %IACS during the second aging, when the first aging was at the temperature of 800°F (427°C). At 12 hours into the second aging, the YS was 621 MPa (90.2 ksi) and the conductivity was 45 %IACS. After 18 hours, the YS had fallen to 432 MPa (65.5 ksi), but the conductivity had increased to 52.8 %IACS.

**FIG. 4** shows the measured YS and %IACS during the second aging, when the first aging was at the temperature of 815°F (435°C). At 12 hours, the YS was 595 MPa (86.4 ksi) and the conductivity was measured at 47.3 %IACS. At 18 hours, the YS was 597 MPa (86.6 ksi) and the conductivity was measured at 51 %IACS.

**FIG. 5** shows the measured YS and %IACS during the second aging, when the first aging was at the temperature of 825°F (441°C). At 12 hours, the YS was 62 MPa (79 ksi) and the conductivity was measured at 48.4 %IACS. At 18 hours, the YS was 506 MPa (73.5 ksi) and the conductivity was measured at 50.5 %IACS.

Selected results for the tensile and conductivity tests are in Table 1 below. Longer aging at 427°C (800°F) resulted in higher conductivity as measured by %IACS and decreased 0.2% offset yield strength.

**Table 1.**

| Alloy | Temp. °C (°F) | Time (hours) | UTS MPa (ksi) | YS MPa (ksi) | %TE | % IACS | Resistivity (µΩ-cm) |
|---|---|---|---|---|---|---|---|
| Cu-Ni-Si-Cr-Mn-Zr | 427 (800) | 12 | 662 (96.1) | 619 (89.8) | 7.88 | 43.6* | 3.96 |
| Cu-Ni-Si-Cr-Mn-Zr | 427 (800) | 12 | 662 (96.1) | 622 (90.3) | 8.36 | 46.3* | 3.73 |
| Cu-Ni-Si-Cr-Mn-Zr | 427 (800) | 18 | 539 (78.2) | 451* (65.4) | 11.39 | 52.9 | 3.26 |
| Cu-Ni-Si-Cr-Mn-Zr | 427 (800) | 18 | 542 (78.7) | 453* (65.7) | 13.13 | 52.8 | 3.27 |
| Cu-Ni-Si-Cr-Mn-Zr | 427 (800) | 24 | 522 (75.8) | 431* (62.6) | 12.33 | 54.8 | 3.15 |
| Cu-Ni-Si-Cr-Mn-Zr | 427 (800) | 24 | 537 (78) | 444* (64.4) | 12.31 | 53.4 | 3.23 |
| Cu-Ni-Si-Cr-Mn-Zr | 435 (815) | 3 | 652 (94.6) | 624 (90.5) | 7.27 | 40.6* | 4.24 |
| Cu-Ni-Si-Cr-Mn-Zr | 435 (815) | 3 | 650 (94.4) | 623 (90.4) | 6.81 | 40.5* | 4.25 |
| Cu-Ni-Si-Cr-Mn-Zr | 435 (815) | 6 | 665 (96.5) | 629 (91.3) | 8.07 | 45.0* | 3.84 |
| Cu-Ni-Si-Cr-Mn-Zr | 435 (815) | 6 | 668 (97) | 633 (91.8) | 7.8 | 44.4* | 3.88 |
| Cu-Ni-Si-Cr-Mn-Zr | 435 (815) | 12 | 643 (93.3) | 595 (86.4) | 9.31 | 47.3* | 3.65 |
| Cu-Ni-Si-Cr-Mn-Zr | 435 (815) | 12 | 645 (93.6) | 595 (86.3) | 6.71 | 47.3* | 3.64 |
| Cu-Ni-Si-Cr-Mn-Zr | 435 (815) | 18 | 525 (76.2) | 427* (62) | 13.15 | 48.7 | 3.54 |
| Cu-Ni-Si-Cr-Mn-Zr | 435 (815) | 18 | 613 (88.9) | 551 (79.9) | 9.53 | 53.8 | 3.20 |
| Cu-Ni-Si-Cr-Mn-Zr | 441 (825) | 18 | 488 (70.8) | 390* (56.6) | 14.374 | 51.7 | 3.33 |
| Cu-Ni-Si-Cr-Mn-Zr | 441 (825) | 18 | 584 (84.8) | 517* (75.1) | 10.64 | 49.3 | 3.49 |

| | | | | | | | |
|---|---|---|---|---|---|---|---|
| *: outside the scope of the invention | | | | | | | |

### REFERENCE EXAMPLE 3¹

A chemical analysis was performed to determine the composition of a Cu-Ni-Si-Cr-Mn-Zr alloy as used herein. The analysis indicated a composition of: <0.01 wt% beryllium, 0.01 wt% cobalt, 1.22 wt% nickel, 0.02 wt% iron, 0.38 wt% silicon, <0.01 wt% aluminum, <0.01 wt% tin, <0.01 wt% zinc, 0.23 wt% chromium, <0.01 wt% lead, 0.08 wt% manganese, 0.02 wt% zirconium, and balance copper. Amounts listed are reported to the hundredths decimal place. Thus, rounding may affect reported amounts of each element as listed herein.

### REFERENCE EXAMPLE 4

Strips of the Cu-Ni-Si-Cr-Mn-Zr alloy described in Reference Example 3 were rolled to 0.2 mm (0.008 inches). The alloy strips were then aged at approximately 454 °C (850°F) for three hours. Ultimate tensile strength (UTS) in MPa (ksi), 0.2% offset yield strength (YS) in MPa (ksi), percent elongation to break (%TE), conductivity (measured by %IACS and resistivity), and hardness were assessed for the Cu-Ni-Si-Cr-Mn-Zr alloy, as well as three other copper alloys: C18150 (Cu-1.0Cr-0.25Zr); C18140M (Cu-0.6Cr-0.1Ag-0.1Ni-0.07Si); and C18070 (Cu-0.7Cr-0.1Ag-0.05Ti-0.02Si). The results are outlined in Table 2 below. The Cu-Ni-Si-Cr-Mn-Zr alloy had improved tensile strength and 0.2% offset yield strength when compared with the other alloys tested. The alloy of the present disclosure also had increased resistivity and hardness compared with the other alloys.

**Table 2.**

| **Alloy** | **UTS MPa (ksi)** | **YS MPa (ksi)** | **%TE** | **%IACS** | **Resistivity (µΩ-cm)** | **Avg. Hardness (HV)** |
|---|---|---|---|---|---|---|
| C18150 | 451 (66.5) | 422 (61.2) | 4.31 | 57.7 | 2.99 | |
| C18150 | 450 (65.3) | 437 (63.4) | 1.331 | 66.3 | 2.6 | 153.0 |
| C18140M | 442 (64.2) | 415 (60.2) | 5.09 | 68.9 | 2.5 | |
| C18140M | 430 (62.4) | 400 (58.1) | 5.44 | 72.4 | 2.38 | 153.6 |
| Cu-Ni-Si-Cr-Mn-Zr | 515 (74.8) | 481 (69.8) | 3.17 | 45.8 | 3.76 | |
| Cu-Ni-Si-Cr-Mn-Zr | 531 (77.1) | 508 (73.8) | 1.824 | 41.0 | 4.21 | 196.0 |
| C18070 | 479 (69.5) | 457 (66.3) | 3.51 | 72.8 | 2.37 | |
| C18070 | 459 (66.6) | 438 (63.5) | 2.51 | 72.5 | 2.38 | 160.3 |

| | | | | | | |
|---|---|---|---|---|---|---|
| ¹ The Reference Examples are outside the scope of the invention | | | | | | |

### REFERENCE EXAMPLE 5

Samples of C18140M (Cu-0.6Cr-0.1Ag-0.1Ni-0.07Si) alloy, Cu-Ni-Si-Cr-Mn-Zr (composition amounts in Reference Example 3), C18070 (Cu-0.7Cr-0.1Ag-0.05Ti-0.02Si) alloy, and C18150 (Cu-1.0Cr-0.5Zr) alloy were cold-worked to a %CW of 70%. Ultimate tensile strength, 0.2% offset yield, and % elongation were measured at room temperature. Each alloy was in the form of a long strip, which was coiled up. Measurements were taken at the inner diameter (ID) and the outer diameter (OD) of each strip, corresponding to the beginning of the casting run (ID) and the end of the casting run (OD). The results of these tests are listed in Table 3 below. After annealing, the alloy of the present disclosure had an ultimate tensile strength greater than that of the other alloys except the Cu-1.0Cr-0.5Zr ID alloy. The yield strength and percent elongation were also similar to the other alloys post-annealing.

The alloys were then aged in a furnace at 454 °C (850°F)REFERENCE for three hours. The samples were water quenched upon removal from the furnace. Results of strength and conductivity testing is listed in Table 3. All alloys had improved ultimate tensile strength when rolled and aged as compared to post-annealing. The Cu-Ni-Si-Cr-Mn-Zr alloy had the highest tensile strength as compared with the other alloys. The alloy also had the lowest %IACS and highest resistivity compared with the other alloys. The alloy of the present disclosure was the only alloy to exhibit 0.2% offset yield strength of at least 551 MPa (80 ksi).

**Table 3.**

| **Alloy** | **Condition** | **UTS MPa (ksi)** | **YS MPa (ksi)** | **%TE** | **%IACS** | **Resistivity (µΩ-cm)** |
|---|---|---|---|---|---|---|
| C18140M ID | Annealed | 267 (38.8) | 76 (11.02) | 43.0 | | |
| C18140M OD | Annealed | 270 (39.2) | 246 (35.7) | 48.0 | | |
| C18140M9 | Rolled/Aged | 487 (70.7) | 449 (65.2) | 9.46 | 77.4 | 2.23 |
| C18140M | Rolled/Aged | 489 (70.9) | 449 (65.1) | 9.16 | 73.1 | 2.36 |
| Cu-Ni-Si-Cr-Mn-Zr ID | Annealed | 292 (42.4) | 84 (12.23) | 39.4 | | |
| Cu-Ni-Si-Cr-Mn-Zr OD | Annealed | 290 (42.1) | 81 (11.7) | 39.2 | | |
| Cu-Ni-Si-Cr-Mn-Zr | Rolled/Aged | 612 (88.8) | 569 (82.6) | 7.94 | 44.3 | 3.89 |
| Cu-Ni-Si-Cr-Mn-Zr | Rolled/Aged | 615 (89.3) | 570 (82.8) | 8.22 | 39.7 | 4.34 |
| C18070 ID | Annealed | 275 (39.9) | 84 (12.12) | 42.8 | | |
| C18070 OD | Annealed | 269 (39.0) | 78 (10.85) | 33.5 | | |
| C18070 | Rolled/Aged | 512 (74.3) | 475 (68.9) | 8.05 | 76.9 | 2.24 |
| C18070 | Rolled/Aged | 518 (75.2) | 478 (69.4) | 9.54 | 75.7 | 2.28 |
| C18150 ID | Annealed | 376 (54.5) | 105 (15.3) | 40.0 | | |
| C18150 OD | Annealed | 225 (32.7) | 68 (9.8) | 41.3 | | |
| C18150 | Rolled/Aged | 528 (76.6) | 488 (70.8) | 10.82 | 65 | 2.65 |
| C18150 | Rolled/Aged | 517 (75.1) | 477 (69.3) | 10.24 | 60.5 | 2.85 |

Hardness of each alloy was also assessed using the Rockwell Hardness 15T Test (15T) and the Vickers Hardness Test (HV). Results are listed in Table 4 below. After annealing, the alloy of the present disclosure had a similar average hardness, as measured by the Rockwell 15T Scale, as the C18150 (Cu-1.0Cr-0.5Zr) alloy. As measured by the Vickers Hardness Test, the Cu-Ni-Si-Cr-Mn-Zr alloy had the highest average hardness post-annealing (as compared with the other alloys post-annealing), and after rolling and aging (as compared with the other alloys after rolling and aging).

**Table 4.**

| **Alloy** | **Condition** | **Avp. Hardness (15T)** | **Avg. Hardness (HV)** |
|---|---|---|---|
| C18140M | Annealed | 51.9 | 88.5 |
| C18140M | Rolled/Aged | | 159.7 |
| Cu-Ni-Si-Cr-Mn-Zr | Annealed | 57.4 | 100.0 |
| Cu-Ni-Si-Cr-Mn-Zr | Rolled/Aged | | 199.8 |
| C18070 | Annealed | 52.3 | 89.8 |
| C18070 | Rolled/Aged | | 168.3 |
| C18150 | Annealed | 58.3 | 92.7 |
| C18150 | Rolled/Aged | | 177.5 |

### REFERENCE EXAMPLE 6

Four samples of the Cu-Ni-Si-Cr-Mn-Zr (composition amounts in Reference Example 3) alloy were placed in a furnace at 427 °C (800°F). After three hours, two of the samples were removed from the furnace and water quenched. The other two samples were removed from the furnace after a total of six hours and subsequently water quenched. Several properties were assessed after processing and aging, including ultimate tensile strength, yield strength, %TE, %IACS, hardness, and resistivity. Results of these tests are in Table 5 below. Aging the alloy for six hours resulted in ultimate tensile strength measurements of 643 and 640 MPa (93.3 and 92.8 ksi), 0.2% offset yield measurements of 603 and 601 MPa (87.5 and 87.2 ksi), and average hardness of 198.9 HV. Additionally, six hours of aging resulted in the alloy having resistivity measurements of 3.91 µΩ-cm and 3.88 µΩ-cm.

**Table 5.**

| **Alloy** | **Temp. °C (°F)** | **Time (hours)** | **UTS MPa (ksi)** | **YS MPa (ksi)** | **%TE** | **%IACS** | **Avg. Hardness (HV)** | **Resistivity (µΩ-cm)** |
|---|---|---|---|---|---|---|---|---|
| Cu-Ni-Si-Cr-Mn-Zr | 427 (800) | 3 | 616 (89.4) | 582 (84.5) | 7.02 | 40.5 | | 4.26 |
| Cu-Ni-Si-Cr-Mn-Zr | 427 (800) | 3 | 626 (90.8) | 587 (85.2) | 7.77 | 39.7 | 187.1 | 4.34 |
| Cu-Ni-Si-Cr-Mn-Zr | 427 (800) | 6 | 643 (93.3) | 603 (87.5) | 8.02 | 44.1 | | 3.91 |
| Cu-Ni-Si-Cr-Mn-Zr | 427 (800) | 6 | 639 (92.8) | 601 (87.2) | 7.63 | 44.5 | 198.9 | 3.88 |

### REFERENCE EXAMPLE 7

Six samples of the Cu-Ni-Si-Cr-Mn-Zr (composition amounts in Reference Example 3) alloy were placed in a furnace at 441 °C (825°F). Two samples were removed at each of the intervals of three, six, and twelve hours and water quenched upon removal. Several properties were assessed including ultimate tensile strength, yield strength, elongation, %IACS, hardness, and resistivity. Results for these tests are listed in Table 6 below. Ultimate tensile strength and yield strength tended to decrease with longer aging. %IACS tended to increase with longer aging. After aging 6 hours, the alloy had the highest average hardness as measured by the Vickers Hardness Test. Resistivity tended to decrease with longer aging.

**Table 6.**

| **Alloy** | **Temp. °C (°F)** | **Time (hours)** | **UTS MPa (ksi)** | **YS MPa (ksi)** | **%TE** | **%IACS** | **Avg. Hardness (HV)** | **Resistivity (µΩ-cm)** |
|---|---|---|---|---|---|---|---|---|
| Cu-Ni-Si-Cr-Mn-Zr | 441 (825) | 3 | 661 (95.9) | 619 (91) | 7.43 | 43.1 | | 4.00 |
| Cu-Ni-Si-Cr-Mn-Zr | 441 (825) | 3 | 661 (96) | 619 (91) | 9.06 | 43.7 | 197.1 | 3.94 |
| Cu-Ni-Si-Cr-Mn-Zr | 441 (825) | 6 | 648 (94) | 601 (87.2) | 9.8 | 46.5 | | 3.71 |
| Cu-Ni-Si-Cr-Mn-Zr | 441 (825) | 6 | 652 (94.7) | 608 (88.3) | 8.16 | 46.1 | 205.3 | 3.74 |
| Cu-Ni-Si-Cr-Mn-Zr | 441 (825) | 12 | 605 (88.9) | 548 (79.6) | 10.41 | 48.5 | | 3.55 |
| Cu-Ni-Si-Cr-Mn-Zr | 441 (825) | 12 | 640 (92.9) | 540 (78.4) | 9.1 | 48.2 | 197.2 | 3.58 |

### REFERENCE EXAMPLE 8

Four samples of the Cu-Ni-Si-Cr-Mn-Zr (composition amounts in Reference Example 3) alloy were cold worked and annealed. The samples were placed in a furnace at 441 °C (825°F) for six hours. Then, the furnace temperature was lowered to 427 °C (800°F), which took 30 minutes to 60 minutes. Two of the samples remained in the furnace for an additional six hours after the 441 °C (825°F) heating, totaling twelve hours time-in-furnace. The remaining two samples remained in the furnace for twelve hours after the 441 °C (825°F) heating, totaling eighteen hours time-in-furnace. Tensile strength, hardness (average of five measurements), and conductivity were assessed and the results are listed in Table 7 below. At 12 hours aging, the alloy had 0.2% offset yield strength measurements of 573 and 574 MPa (83.1 ksi and 83.3 ksi), the alloy had conductivity of 49.3% IACS and 49.1 IACS. Longer aging tended to result in lower ultimate tensile strength, yield strength, and hardness. Eighteen hours of aging resulted in increased resistivity and percent elongation as compared with 12 hours. At both 12 and 18 hours of aging, the alloy had greater than 48% IACS.

**Table 7.**

| **Alloy** | **Time (hours)** | **UTS MPa (ksi)** | **YS MPa (ksi)** | **%TE** | **%IACS** | **Avg. Hardness (HV)** | **Resistivity (µΩ-cm)** |
|---|---|---|---|---|---|---|---|
| Cu-Ni-Si-Cr-Mn-Zr | 12 | 628 (91.2) | 573 (83.1) | 9.69 | 49.3 | | 3.50 |
| Cu-Ni-Si-Cr-Mn-Zr | 12 | 632 (91.7) | 574 (83.3) | 9.39 | 49.1 | 199.1 | 3.51 |
| Cu-Ni-Si-Cr-Mn-Zr | 18 | 599 (86.9) | 529 (76.8) | 10.06 | 48.7 | | 3.54 |
| Cu-Ni-Si-Cr-Mn-Zr | 18 | 600 (87.1) | 533 (77.4) | 9.9 | 51.6 | 187.9 | 3.34 |

### COMPARATIVE EXAMPLE 9

Four samples of each of C18140M (Cu-0.Cr-0.1Ag-0.1Ni-0.07Si), C18070 (Cu-0.7Cr-0.1Ag-0.05Ti-0.02Si), and C18150 (Cu-1.0Cr-0.25Zr) alloys were cut. Conductivity and tensile measurements were taken on the as-received alloys. The remaining samples were then heated for three hours at 441 °C (825°F). Tensile strength and conductivity measurements were then taken on these samples. Results of these tests are listed in Table 8 below. None of the alloys tested had a 0.2% offset yield strength of at least 551 MPa (80 ksi). Only after aging did the alloys have a conductivity of at least 48% IACS.

**Table 8.**

| **Alloy** | **Temp. °C (°F)** | **Time (hours)** | **UTS MPa (ksi)** | **YS MPa (ksi)** | **%TE** | **%IACS** | **Resistivity (µΩ-cm)** |
|---|---|---|---|---|---|---|---|
| C18140M ID | N/A | N/A | 463 (67.2) | 446 (64.8) | 1.432 | 39.2 | 4.4 |
| C18140M OD | N/A | N/A | 469 (68) | 450 (65.3) | 1.375 | 40.7 | 4.24 |
| C18070 ID | N/A | N/A | 477 (69.2) | 460 (66.8) | 1.573 | 32.7 | 5.27 |
| C18070 OD | N/A | N/A | 500 (72.6) | 457 (66.4) | 1.766 | 34.5 | 5.00 |
| C18150 | N/A | N/A | 502 (72.9) | 478 (69.4) | 1.843 | 34.5 | 5.00 |
| C18150 | N/A | N/A | 491 (71.3) | 469 (68) | 2.09 | 34.2 | 5.03 |
| C18140M | 441 (825) | 3 | 503 (73) | 468 (67.9) | 7.79 | 69.6 | 2.48 |
| C18140M | 441 (825) | 3 | 511 (74.2) | 472 (68.5) | 6.7 | 76.2 | 2.26 |
| C18070 | 441 (825) | 3 | 542 (78.7) | 515 (74.8) | 7.6 | 76.9 | 2.24 |
| C18070 | 441 (825) | 3 | 538 (78.1) | 506 (73.4) | 7.99 | 70.7 | 2.44 |
| C18150 | 441 (825) | 3 | 539 (78.2) | 507 (73.6) | 8.44 | 69.6 | 2.48 |
| C18150 | 441 (825) | 3 | 539 (78.3) | 508 (73.7) | 8.48 | 64.4 | 2.68 |

### COMPARATIVE EXAMPLE 10

Two samples of C18070 (Cu-0.7Cr-0.1Ag-0.05Ti-0.02Si) alloy of approximately 0.008 inch thickness were heat treated for six hours. One of the samples was heat treated at 441 °C (825°F). The other sample was heat treated at 427 °C (800°F). Upon removal from the furnace, both were water quenched, and their tensile and conductivity properties were assessed.

Eight samples of C18150 (Cu-1.0Cr-0.25Zr) alloy were taken and heat treated as follows: two were heated at 482 °C (900°F) for one hour and water quenched; two were heated at 482 °C (900°F) for two hours and water quenched; two were heated at 496 °C (925°F) for one hour and water quenched; two were heated at 496 °C (925°F) for two hours and water quenched. Conductivity and tensile measurements were taken. The results are summarized in Table 9 below. None of the alloys tested had a 0.2% offset yield strength of at least 551 MPa (80 ksi). All alloys tested had a conductivity greater than 48% IACS.

**Table 9.**

| **Alloy** | **Temp. °C (°F)** | **Time (hours)** | **UTS MPa (ksi)** | **YS MPa (ksi)** | **%TE** | **%IACS** | **Resistivity (µΩ-cm)** |
|---|---|---|---|---|---|---|---|
| C18070 | 441 (825) | 6 | 520 (75.5) | 500 (72.5) | 9.79 | 79.0 | 2.18 |
| C18070 | 423 (800) | 6 | 517 (75.1) | 496 (72) | 8.29 | 80.8 | 2.13 |
| C18150 | 482 (900) | 1 | 533 (77.3) | 495 (71.8) | 8.93 | 63.0 | 2.74 |
| C18150 | 482 (900) | 1 | 539 (78.2) | 502 (72.8) | 9.63 | 64.9 | 2.66 |
| C18150 | 482 (900) | 2 | 524 (76) | 482 (69.9) | 9.24 | 64.2 | 2.69 |
| C18150 | 482 (900) | 2 | 517 (75) | 473 (68.7) | 9.62 | 66.6 | 2.59 |
| C18150 | 496 (925) | 1 | 521 (75.6) | 480 (69.6) | 10.51 | 61.9 | 2.79 |
| C18150 | 496 (925) | 1 | 517 (75.1) | 476 (69.1) | 8.64 | 65.6 | 2.63 |
| C18150 | 496 (925) | 2 | 490 (71.1) | 440 (63.8) | 9 | 66.4 | 2.60 |
| C18150 | 496 (925) | 2 | 491 (71.3) | 440 (63.9) | 10.11 | 62.7 | 2.75 |

### EXAMPLE 11

Strips comprising from 1.2 wt% to 1.4 wt% nickel; from 0.3 wt% to 4 wt% silicon; from 0.3 wt% to 0.4 wt% chromium; from 0.08 wt% to 0.12 wt% manganese; from 0.02 wt% to 0.06 wt% zirconium; and balance copper were made according to the present disclosure and tested.

The alloys were cold worked and annealed. The samples were placed in a furnace at 441 °C (825°F) for six hours. Then, the furnace temperature was lowered to 427 °C (800°F), which took 30 minutes to 60 minutes. The samples were then heated for an additional six hours after the 441 °C (825°F) heating, totaling twelve hours time-in-furnace. The ultimate tensile strength (UTS), 0.2% offset yield strength (YS), total elongation to break (%TE), elastic modulus (EM), electrical conductivity (%lACS)Several properties were measured (UTS, Yield Strength, and the formability in both directions (GW, BW). The results are listed in Table 10 below, as well as the gauge for each strip.

**Table 10.**

| **Alloy** | **Gauge cm (in)** | **UTS MPa (ksi)** | **YS MPa (ksi)** | **%TE** | **EM GPa (Msi)** | **%IACS** | **GW** | **BW** |
|---|---|---|---|---|---|---|---|---|
| Cu-Ni-Si-Cr-Mn-Zr | 0.08 (0.0315) | 666 (96.6) | 617 (89.5) | 9.7 | 148 (21.4) | 49.5 | 0.10 | 0.30 |
| Cu-Ni-Si-Cr-Mn-Zr | 0.06 (0.0236) | 670 (97.2) | 617 (89.5) | 9.7 | 141 (20.5) | 49.0 | 0.10 | 0.50 |
| Cu-Ni-Si-Cr-Mn-Zr | 0.02 (0.00787) | 646 (93.7) | 582 (84.4) | 10 | | 50 | 0.5 | 0.5 |
| Cu-Ni-Si-Cr-Mn-Zr | 0.02 (0.00787) | 628 (91.1) | 586 (85.0) | 8.2 | 150 (21.8) | 50.3 | 0.0 | 0.0 |

## Claims

1. A copper alloy, comprising:
from 1.2 wt% to 1.4 wt% nickel;
from 0.3 wt% to 0.4 wt% silicon;
from 0.3 wt% to 0.4 wt% chromium;
from 0.08 wt% to 0.12 wt% manganese;
from 0.02 wt% to 0.06 wt%zirconium; and
balance copper and unavoidable impurities;
wherein the alloy has a 0.2% offset yield strength of at least 551 MPa and a conductivity of at least 48% IACS.

2. The copper alloy of claim 1, wherein the alloy does not contain beryllium, titanium, iron, cobalt, magnesium, or boron.

3. The copper alloy of claim 1, wherein the alloy has an ultimate tensile strength of at least 606 MPa.

4. The copper alloy of claim 1, wherein the alloy has an elastic modulus of at least 137,895 MPa.

5. The copper alloy of claim 1, wherein the alloy has a % total elongation of at least 8%.

6. The copper alloy of claim 1, wherein the alloy has a ductility of at least 5% to about 15%.

7. The copper alloy of claim 1, wherein the alloy has a formability ratio of 0.4/1 or lower.

8. The copper alloy of claim 1, containing silicides formed from silicon, chromium, nickel, and manganese.

9. The copper alloy of claim 1, having a 0.2% offset yield strength of at least 551 MPa, a conductivity of at least 48% IACS, and a % total elongation to break of at least 8%.

10. The copper alloy of claim 1, having a 0.2% offset yield strength of at least 551 MPa, a conductivity of at least 49% IACS, and a ultimate tensile strength of at least 620 MPa.

11. A process to obtain the copper alloy of claim 1 that does not contain beryllium and has a 0.2% offset yield strength of at least 551 MPa and a conductivity of at least 48% IACS, comprising:
cold working a copper-nickel-silicon-chromium-manganese-zirconium alloy to a percentage of cold working (% CW) of 80% to 95%;
solution annealing the cold-worked copper-nickel-silicon-chromium-manganese-zirconium alloy; and
aging the solution-annealed copper-nickel-silicon-chromium-manganese-zirconium alloy to obtain the copper alloy with a 0.2% offset yield strength of at least 551 MPa and a conductivity of at least 48% IACS.

12. The process of claim 11, wherein the solution annealing is performed at a temperature of 900°C to 1000°C for a time period of 5 minutes to 20 minutes.

13. The process of claim 11, wherein the aging is performed at a temperature of 400°C to 460°C for a time period of 6 hours to 60 hours, preferably for a time period of 6 hours to 18 hours.

14. An article formed from the copper alloy of claim 1, wherein the article is a heat sink; an electrical connector; an electronic connector; a wiring harness terminal; an electric vehicle charger contact; a high voltage/current/power terminal contact; a power connector contact; a midplane connector; a backplane connector; a card edge connector; a photovoltaic system connector; an appliance power contact; a computer power contact; a heat spreader; a bushing or bearing surface; or a component for an electronic device or an electrical device.

## Patentansprüche

1. Kupferlegierung, umfassend:
von 1,2 Gew.-% bis 1,4 Gew.-% Nickel,
von 0,3 Gew.-% bis 0,4 Gew.-% Silicium,
von 0,3 Gew.-% bis 0,4 Gew.-% Chrom,
von 0,08 Gew.-% bis 0,12 Gew.-% Mangan,
von 0,2 Gew.-% bis 0,06 Gew.-% Zirconium, und
ansonsten Kupfer und unvermeidliche Verunreinigungen,
wobei die Legierung eine 0,2%-Dehngrenze von wenigstens 551 MPa und eine Leitfähigkeit von wenigstens 48% IACS aufweist.

2. Kupferlegierung nach Anspruch 1, wobei die Legierung kein Beryllium, Titan, Eisen, Cobalt, Magnesium oder Bor enthält.

3. Kupferlegierung nach Anspruch 1, wobei die Legierung eine Zugfestigkeit von wenigstens 606 MPa aufweist.

4. Kupferlegierung nach Anspruch 1, wobei die Legierung ein Elastizitätsmodul von wenigstens 137,895 MPa aufweist.

5. Kupferlegierung nach Anspruch 1, wobei die Legierung eine Bruchdehnung von wenigstens 8% aufweist.

6. Kupferlegierung nach Anspruch 1, wobei die Legierung eine Duktilität von wenigstens 5% bis ungefähr 15% aufweist.

7. Kupferlegierung nach Anspruch 1, wobei die Legierung ein Formbarkeitsverhältnis von 0,4/1 oder weniger aufweist.

8. Kupferlegierung nach Anspruch 1, das Silicide aus Silicium, Chrom, Nickel und Mangan enthält.

9. Kupferlegierung nach Anspruch 1, das eine 0,2%-Dehngrenze von wenigstens 551 MPa, eine Leitfähigkeit von wenigstens 48% IACS und eine Bruchdehnung von wenigstens 8% aufweist.

10. Kupferlegierung nach Anspruch 1, das eine 0,2%-Dehngrenze von wenigstens 551 MPa, eine Leitfähigkeit von wenigstens 49% IACS und eine Zugfestigkeit von wenigstens 620 MPa aufweist.

11. Verfahren zum Erhalten einer Kupferlegierung nach Anspruch 1, das kein Beryllium enthält, eine 0,2%-Dehngrenze von wenigstens 551 MPa und eine Leitfähigkeit von wenigstens 48% IACS aufweist, umfassend:
Kaltumformen einer Kupfer-Nickel-Silicium-Chrom-Mangan-Zirconium-Legierung zu einem Prozentsatz einer Kaltumformung (% CW) von 80% bis 95%,
Lösungsglühen der kaltumgeformten Kupfer-Nickel-Silicium-Chrom-Mangan-Zirconium-Legierung, und
Aushärten der lösungsgeglühten Kupfer-Nickel-Silicium-Chrom-Mangan-Zirconium-Legierung, um die Kupferlegierung mit einer 0,2%-Dehngrenze von wenigstens 551 MPa und einer Leitfähigkeit von wenigstens 48% IACS zu erhalten.

12. Verfahren nach Anspruch 11, wobei das Lösungsglühen bei einer Temperatur von 900°C bis 1000°C für eine Zeitdauer von 5 Minuten bis 20 Minuten durchgeführt wird.

13. Verfahren nach Anspruch 11, wobei das Aushärten bei einer Temperatur von 400°C bis 460°C für eine Zeitdauer von 6 Stunden bis 60 Stunden und vorzugsweise eine Zeitdauer von 6 Stunden bis 18 Stunden durchgeführt wird.

14. Artikel, der aus der Kupferlegierung des Anspruchs 1 ausgebildet ist, wobei der Artikel eine Wärmesenke, ein elektrischer Steckverbinder, ein elektronischer Steckverbinder, ein Kabelbaumanschluss, ein Elektrofahrzeug-Ladekontakt, ein Hochspannung/-strom/-leistung-Anschlusskontakt, ein Stromsteckverbinderkontakt, ein Midplane-Steckverbinder, ein Backplane-Steckverbinder, ein Kartenkanten-Steckverbinder, ein Photovoltaiksystem-Steckverbinder, ein Geräte-Stromkontakt, ein Computer-Stromkontakt, ein Wärmespreizer, eine Buchsen- oder Lageroberfläche oder eine Komponente für ein elektronisches oder ein elektrisches Gerät ist.

## Revendications

1. Alliage de cuivre, comprenant :
de 1,2 % en poids à 1,4 % en poids de nickel ;
de 0,3 % en poids à 0,4 % en poids de silicium ;
de 0,3 % en poids à 0,4 % en poids de chrome ;
de 0,08 % en poids à 0,12 % en poids de manganèse ;
de 0,02 % en poids à 0,06 % en poids de zirconium ; et
le reste étant du cuivre et des impuretés inévitables ;
dans lequel l'alliage a une limite d'élasticité conventionnelle à 0,2 % d'au moins 551 MPa et une conductivité d'au moins 48 % IACS.

2. Alliage de cuivre selon la revendication 1, dans lequel l'alliage ne contient pas de béryllium, de titane, de fer, de cobalt, de magnésium ou de bore.

3. Alliage de cuivre selon la revendication 1, dans lequel l'alliage a une résistance à la traction ultime d'au moins 606 MPa.

4. Alliage de cuivre selon la revendication 1, dans lequel l'alliage a un module d'élasticité d'au moins 137 895 MPa.

5. Alliage de cuivre selon la revendication 1, dans lequel l'alliage a un allongement total en % d'au moins 8 %.

6. Alliage de cuivre selon la revendication 1, dans lequel l'alliage a une ductilité d'au moins 5 % à environ 15 %.

7. Alliage de cuivre selon la revendication 1, dans lequel l'alliage a un rapport de formabilité de 0,4/1 ou moins.

8. Alliage de cuivre selon la revendication 1, contenant des siliciures formés à partir de silicium, de chrome, de nickel et de manganèse.

9. Alliage de cuivre selon la revendication 1, ayant une limite d'élasticité conventionnelle à 0,2 % d'au moins 551 MPa, une conductivité d'au moins 48 % IACS et un allongement total à la rupture en % d'au moins 8%.

10. Alliage de cuivre selon la revendication 1, ayant une limite d'élasticité conventionnelle à 0,2 % d'au moins 551 MPa, une conductivité d'au moins 49 % IACS et une résistance à la traction ultime d'au moins 620 MPa.

11. Procédé d'obtention de l'alliage de cuivre selon la revendication 1 qui ne contient pas de béryllium et a une limite d'élasticité conventionnelle à 0,2 % d'au moins 551 MPa et une conductivité d'au moins 48 % IACS, comprenant :
le travail à froid d'un alliage de cuivre-nickel-silicium-chrome-manganèse-zirconium à un pourcentage de travail à froid (% CW) de 80 % à 95 % ;
le recuit de mise en solution de l'alliage de cuivre-nickel-silicium-chrome-manganèse-zirconium travaillé à froid ; et
le vieillissement de l'alliage de cuivre-nickel-silicium-chrome-manganèse-zirconium ayant été soumis au recuit de mise en solution pour obtenir l'alliage de cuivre ayant une limite d'élasticité conventionnelle à 0,2 % d'au moins 551 MPa et une conductivité d'au moins 48 % IACS.

12. Procédé selon la revendication 11, dans lequel le recuit de mise en solution est réalisé à une température de 900 °C à 1 000 °C pendant une durée de 5 minutes à 20 minutes.

13. Procédé selon la revendication 11, dans lequel le vieillissement est effectué à une température de 400 °C à 460 °C pendant une période de 6 heures à 60 heures, de préférence pendant une période de 6 heures à 18 heures.

14. Article formé à partir de l'alliage de cuivre selon la revendication 1, dans lequel l'article est un dissipateur thermique ; un connecteur électrique ;
un connecteur électronique ; une borne de faisceau de câblage ; un contact de chargeur de véhicule électrique ; un contact de borne haute tension/courant/puissance ; un contact de connecteur d'alimentation ; un connecteur de plan médian ; un connecteur de plan de fond ; un connecteur de bord de carte ; un connecteur de système photovoltaïque ; un contact d'alimentation d'appareil ; un contact d'alimentation d'ordinateur ; un dissipateur thermique ; une douille ou une surface d'appui ; ou un composant pour un dispositif électronique ou un dispositif électrique.
